

## UNITED STATES PATENT OFFICE

2,045,346

MANUFACTURE OF ARTIFICIAL SILK AND  
OTHER ARTIFICIAL PRODUCTS

Henry Dreyfus, London, and William Ivan Taylor, Spondon, near Derby, England, assignors to Celanese Corporation of America, a corporation of Delaware

No Drawing. Application July 1, 1932, Serial No. 620,543. In Great Britain August 19, 1931

13 Claims. (Cl. 18—54)

This invention relates to the manufacture of filaments, threads, yarns and the like from solutions of cellulose acetate or other cellulose esters or ethers by the dry spinning or evaporative method.

It is well known that in the early days of the cellulose acetate artificial silk industry considerable difficulties arose from the fact that fabrics made from such filaments exhibited the disadvantage of scintillation, and it was found that this was due at least in part to the relatively flat cross-section which the filaments exhibited. These difficulties were overcome to a large extent by the use of spinning solutions containing upwards of 20%, and particularly 25% or more, of cellulose acetate, (see U. S. Patent No. 1,688,531). The present invention is likewise concerned with methods for improving the cross-section of the filaments. We have found, and this forms the basis of the present invention, that a spinning solution containing a volatile constituent in addition to the liquid forming the main bulk of the solvent or solvent mixture is capable of yielding filaments which are very much rounder than the filaments obtained from such a solution in the absence of the volatile constituent.

According to the present invention, therefore, artificial filaments, threads, yarns and the like of improved cross-section are obtained by dry spinning processes from solutions containing a volatile constituent in addition to the solvent or solvent mixture forming the main bulk of the spinning solution.

The volatile agents employed for the purpose of the present invention may be solvents for the cellulose derivative, as for example methyl or ethyl formate in the case of acetone-soluble cellulose acetate spun from acetone solutions, latent solvents, that is to say substances which are practically solvents, as for example methylene chloride in the case of acetone-soluble cellulose acetate, weakly acting precipitants or substances which are swelling or gelling agents for the cellulose derivatives, or strongly acting precipitants for the cellulose derivative. Precipitants, and especially strongly acting precipitants, are the most useful liquids for the purposes of the present invention. In this last category we have found that the ethers, and particularly diethyl ether, are especially valuable. Other ethers which may be employed are methyl or ethyl propyl ether, ethyl isopropyl ether and di-isopropyl ether. Furthermore the low boiling fractions of petroleum, and particularly petrol ether or fractions thereof, and also the lower fractions of

gasoline and other low boiling hydrocarbons, may be employed.

The volatile liquid may be added in any suitable proportion in relation to the cellulose derivative or to the main bulk of solvent or solvent mixture used. In employing non-solvents it will be appreciated that the proportion of volatile liquid to be added is limited by considerations of the solubility of the cellulose derivative in the mixture of solvent and volatile liquid. We have obtained very good results by dissolving an acetone-soluble cellulose acetate in a mixture consisting of 6 to 12% of diethyl ether and 94 to 88% of acetone. Similar proportions may be used in the case of petrol ether, though it has been found that proportions of 10% and under, down to 2% or even less, are preferable.

If water be included in a spinning solution containing a solvent or solvent mixture miscible therewith, we find that the draw-down of the filaments is thereby improved. Similarly methyl or ethyl alcohol and like liquids will improve the draw-down, though to a less extent than water. The present invention therefore envisages the spinning of a solution containing, in addition to the main bulk of solvent or solvent mixture and the volatile liquid characteristic of the invention, a proportion, for example 3 to 5% or even up to 10%, of water or other liquid adapted to improve the draw-down of the filaments. For instance, we have obtained highly satisfactory results by dissolving an acetone-soluble cellulose acetate in a mixture containing 86% of acetone, 6% of water and 8% of diethyl ether.

The process of the present invention is capable of being applied to spinning solutions of all kinds, and the invention is not limited to acetone solutions of acetone-soluble cellulose acetates which have been more particularly discussed above. Other cellulose esters, as for example cellulose formate, cellulose propionate, cellulose butyrate and the like and mixed esters, for example cellulose acetate-butyrate and cellulose nitro-acetate, and also cellulose ethers, as for example ethyl or benzyl cellulose, ethyl-benzyl cellulose or other mixed ethers and mixed ether-esters of cellulose, may be employed. Further, instead of using acetone as the solvent or the main bulk of the solvent, mixtures of acetone and alcohol, acetone and methyl alcohol, ethyl or methyl acetate and ethyl or methyl alcohol, or mixtures of any of these solvents may be employed, or indeed any other suitable solvents. The invention improves the cross-section of the filaments no matter what concentra-

tion of spinning solution may be employed, that is to say that even when employing concentrations of 25% or higher in the spinning solution, improved cross-sections are obtainable. However, the maximum advantage of the present invention is attained in the case of spinning filaments from solutions of lower concentration, as for example 25 to 20 or 15% or less by weight of the cellulose derivative. The ability to improve the cross-sections of filaments obtainable from these lower concentrations is of especial advantage in the case of spinning at the modern high speeds, such as 200 to 300 or 400 or more metres per minute, though advantages still accrue from the employment of the older lower spinning speeds, such as 150 or 100 metres per minute. With the higher spinning speeds it is found that the draw-down of the filaments is not as good as in the case of spinning the same spinning solutions through the same jet orifices at lower spinning speeds, which is a disadvantage in view of the commercial demand for low filament deniers. By enabling filaments of round cross-section to be obtained from solutions of relatively low concentration, the present invention makes it possible to obtain low filament deniers of good cross-section at the modern high spinning speeds, and the process of the invention is therefore extremely valuable in this connection.

In order to improve still further the cross-section and other valuable characteristics of the filaments cellulose derivatives, and particularly cellulose acetates, of high viscosity characteristics, for example those obtained by the process described in U. S. Patent No. 1,829,822, may be used. The present invention includes therefore the use of these cellulose derivatives in the special spinning solutions described above.

Furthermore, we have found that for the purpose of obtaining good cross-sections it is of great importance to promote a rapid evaporation in the very early stages of spinning by the dry spinning method. For example, we have found that if a rapid evaporation of the solvent or solvent mixture be brought about within the first two inches of the travel of the filaments through the usual dry spinning cell, better cross-sections are obtainable than if evaporation is allowed to proceed normally. The figure of two inches is given in relation to the usual type of dry spinning cell in which the travel of the filaments is about six or seven feet within the spinning cell. The figure appears to be critical, since a rapid evaporation at a distance of three inches from the nozzle does not produce the same effect. It is probably for this reason that the ethers and other highly volatile liquids have a beneficial effect upon the cross-section of the filaments. In order to improve this effect still further other means may be adopted to induce a rapid evaporation in the very early stages of the spinning. For example, it is of great advantage to cause a current of evaporative medium to cross the face of the nozzle or otherwise introduce fresh evaporative medium in the immediate vicinity of the nozzle; (compare U. S. application S. No. 382,907 filed 2nd August, 1929). The evaporative medium so introduced may be heated or not and may be directed towards the filaments from one side only or from two or more points of the spinning cell or from the centre of the nozzle so as to blow across the filaments in a radial direction when employing jet orifices arranged in a ring, as in the ring

type or disc type nozzle. Furthermore, greater evaporation may be induced by employing the collector devices of U. S. applications S. Nos. 236,448 filed 29th November, 1927, 311,213 filed 8th October, 1928, 311,214 filed 8th October, 1928, 5 405,784 filed 8th November, 1929, and 495,140 filed 12th November, 1930. Again a very rapid evaporation in the early stages of spinning may be achieved by employing a vacuum or sub-atmospheric pressure in the spinning cell or chamber as described and claimed in U. S. application S. No. 375,150 filed 1st July, 1929. A combination of two or more of the above devices may be effected in order to improve still further the evaporation. 15

All the above advantages of the present invention may be obtained by means of jet orifices of the normal size, for example .05 to .08 or .10 millimetre diameter. Jet orifices of larger cross-section or of smaller cross-section down to the minimum obtainable may, however, be used.

The following examples are given to illustrate the invention, but it is to be clearly understood that they do not limit it in any way.

#### Example 1

A solution of cellulose acetate, of about 20-21% concentration, in an acetone-diethyl ether mixture containing about 88% of acetone and 12% of diethyl ether is spun through jets of .055 millimetre diameter at a spinning speed of from 200-250 metres per minute. Filaments of low denier, for example, from 2-3 deniers having a good cross-section are obtained.

#### Example 2

A cellulose acetate solution of from 22-23% concentration in a mixture consisting of about 8% diethyl ether, 86% acetone and 6% water is spun under similar conditions to those obtaining in Example 1, and filaments of low denier and good cross-section are obtained.

#### Example 3

A 22-24% solution of cellulose acetate in a mixture consisting of about 93% acetone, 5% water and 2% petroleum ether, of a boiling range of 40-60° C., is spun under similar conditions to those of the previous examples and similar products are obtained.

#### Example 4

A 23-26% solution of cellulose acetate in a solvent mixture consisting of from 6-10% isopropyl ether and 94-90% acetone is spun through jets of .07 millimetre diameter at a speed of 150-200 metres per minute, yielding filaments of improved cross-section.

The invention has been described above more particularly in relation to the manufacture of filaments, in which it is of the greatest value. Nevertheless advantages accrue by employing the process of the invention for the manufacture of other types of products, for example ribbons.

What we claim and desire to secure by Letters Patent is:—

1. Process for the production of solid artificial filaments, threads and the like of improved bulbous cross-section, which comprises forming a 70 solution of an organic derivative of cellulose in a solvent mixture comprising a liquid medium which is a solvent for the organic derivative of cellulose and a smaller proportion of a more volatile non-solvent for the organic derivative of cel- 75

lulose, and extruding said solution through suitable orifices into an evaporative atmosphere.

2. Process for the production of solid artificial filaments, threads and the like of improved bulbous cross-section, which comprises forming a solution of cellulose acetate in a solvent mixture comprising a solvent for the cellulose acetate and not more than 12%, based on the solvent mixture, of a more volatile non-solvent for the cellulose acetate and extruding said solution through suitable orifices into an evaporative atmosphere.

3. Process for the production of solid artificial filaments, threads and the like of improved bulbous cross-section, which comprises forming a solution of an organic derivative of cellulose in a solvent mixture comprising a solvent for the organic derivative of cellulose and not more than 12%, based on the solvent mixture, of an aliphatic ether which is more volatile than the said solvent, and extruding the said solution through suitable orifices into an evaporative atmosphere.

4. Process for the production of solid artificial filaments, threads and the like of improved bulbous cross-section, which comprises forming a solution of cellulose acetate in a solvent mixture comprising a solvent for the cellulose acetate and a smaller proportion of diethyl ether, the said solvent being less volatile than diethyl ether, and extruding said solution through suitable orifices into an evaporative atmosphere.

5. Process for the production of solid artificial filaments, threads and the like of improved bulbous cross-section, which comprises forming a solution of cellulose acetate in a solvent mixture containing acetone and diethyl ether, the proportion of diethyl ether being between 6 and 12% of the solvent mixture, and extruding said solution through suitable orifices into an evaporative atmosphere.

6. Process for the production of solid artificial filaments, threads and the like of improved bulbous cross-section, which comprises forming a solution of an organic derivative of cellulose in an aqueous solvent mixture comprising a solvent for the organic derivative of cellulose and a smaller proportion of an aliphatic ether which is more volatile than the said solvent, and extruding said solution through suitable orifices into an evaporative atmosphere.

7. Process for the production of solid artificial filaments, threads and the like of improved bulbous cross-section, which comprises forming an 18 to 25% solution of cellulose acetate in a solvent mixture comprising acetone and a smaller proportion of diethyl ether, extruding said solution through suitable orifices, and drawing off the products at a speed greater than 150 metres per minute.

8. Process for the production of solid artificial

filaments, threads and the like of improved bulbous cross-section, which comprises forming a solution of cellulose acetate of relatively high viscosity characteristics in a solvent mixture comprising acetone and a smaller proportion of diethyl ether, extruding said solution through suitable orifices and drawing off the products at a speed greater than 150 metres per minute.

9. Process for the production of solid artificial filaments, threads and the like of improved bulbous cross-section, which comprises forming a solution of an organic derivative of cellulose in a solvent mixture comprising a solvent for the organic derivative of cellulose and a smaller proportion of an aliphatic ether which is more volatile than said solvent, extruding the said solution through suitable orifices into an evaporative atmosphere, and inducing rapid evaporation of the solvent mixture near the extrusion orifices.

10. Process for the production of solid artificial filaments, threads and the like of improved bulbous cross-section, which comprises forming a solution of cellulose acetate in a solvent mixture comprising acetone and a smaller proportion of diethyl ether, extruding said solution through suitable orifices into an evaporative atmosphere, and inducing rapid evaporation of the solvent mixture near the extrusion orifices.

11. Process for the production of solid artificial filaments, threads and the like of improved bulbous cross-section, which comprises forming a solution of cellulose acetate in a solvent mixture comprising a solvent for the cellulose acetate and a smaller proportion of a more volatile non-solvent for the cellulose acetate selected from the group consisting of methyl propyl ether, ethyl propyl ether, ethyl isopropyl ether, di-isopropyl ether and petroleum ether fractions boiling above 40° C., and extruding the said solution through suitable orifices into an evaporative atmosphere.

12. Process for the production of solid artificial filaments, threads and the like of improved bulbous cross-section, which comprises forming a solution of cellulose acetate in a solvent mixture comprising acetone and a smaller proportion of methyl propyl ether, and extruding the said solution through suitable orifices into an evaporative atmosphere.

13. Process for the production of solid artificial filaments, threads and the like of improved bulbous cross-section, which comprises forming a solution of cellulose acetate in a solvent mixture comprising acetone and a smaller proportion of a petroleum ether fraction boiling above 40° C. but being more volatile than acetone, and extruding the said solution through suitable orifices into an evaporative atmosphere.

HENRY DREYFUS.  
WILLIAM IVAN TAYLOR. 60